

F. L. BISHOP,  
METHOD OF TREATING METALS,  
APPLICATION FILED FEB. 26, 1913.

1,171,832.

Patented Feb. 15, 1916.



WITNESSES

R. A. Balderson  
A. T. McConville

INVENTOR

F. L. Bishop  
by Clarence Byers & Lamme  
his atty

# UNITED STATES PATENT OFFICE.

FREDERIC L. BISHOP, OF PITTSBURGH, PENNSYLVANIA.

## METHOD OF TREATING METALS.

1,171,832.

Specification of Letters Patent. Patented Feb. 15, 1916.

Application filed February 28, 1913. Serial No. 750,844.

To all whom it may concern:

Be it known that I, FREDERIC L. BISHOP, a citizen of the United States, residing at Pittsburgh, in the county of Allegheny and 5 State of Pennsylvania, have invented a new and useful Method of Treating Metals, of which the following is a full, clear, and exact description, reference being had to the accompanying drawings, in which the 10 figure is a diagrammatic sectional side elevation showing one form of apparatus for carrying out my invention.

Heretofore in changing the molecular structure or size of grain of metals, it has 15 been customary to subject them to heat treatment of mechanical work, or both. Thus, it is well known that in annealing, tempering and hardening processes the heating of the piece, especially beyond certain temperatures, produces a change in structure. Again, simple 20 mechanical work in the way of forging, hammering, rolling, drawing, etc., is known to change the structure of the metal.

I have discovered that by subjecting 25 metal to the action of the magnetic field of an alternating current either with or without heating of the metal, the structure or size of grain of the metal may be altered. In practice, I prefer to so apply the alternating 30 current that the metal will be heated as well as subjected to its magnetic field, since the desired change in structure is much more rapidly produced.

My invention may be applied to any metal 35 in a solid state and the method of applying the magnetic field of the alternating current may be widely varied without departing from my invention.

In the drawings, in which I show one form 40 of apparatus for carrying out my process, 2 represents an alternating current generator whose leads are connected to the primary regulating transformer 3, the leads from the secondary of this transformer are connected 45 to the terminals of coil 4 of bare copper wire, preferably wound around an asbestos cylinder 5 inclosing the bar of steel to be treated. This may, as in this example, be a round bar of steel, say one and a half 50 inches in diameter. The copper wire may have say 300 turns and be of No. 4 size and through it I pass an alternating current of say 50 amperes and preferably 60 alternations per second. In this case the metal bar 55 is heated by the induced eddy currents

therein, as well as acted on by the magnetic field. Under these conditions, the heating of the metal is uniform throughout and the action of the magnetic field in changing the structure is greatly hastened by the heating 60 effect. This treatment is preferably continued, in the example just referred to, until the steel is brought to a temperature lower than that employed in the ordinary annealing of steel. For example, on a steel 65 for which 900° C. is recommended for annealing, I have found that the desired result is obtained by my process when a temperature of 750° to 800° C. is reached. The rate of rise in temperature is, of course, 70 easily controlled and regulated by means of the current and this part of the operation may be easily carried out in less than an hour. The bar is then slowly cooled by gradually decreasing the amount of current 75 or by leaving the bar in the coil and turning off the current.

I preferably surround the article and coil with non-heat conducting material, indicated at 6 in the drawing, to prevent radiation and conduction of heat and make the 80 method more economical.

If a bar of steel is to be hardened or tempered, it may be treated in the same manner as above described, the bar when it has 85 reached the desired condition, as indicated by its magnetic properties or temperature, or both, being withdrawn and quenched or treated in the usual manner for hardening after which it may be returned to the apparatus for further treatment in tempering.

It will be noted that my method is not for mere electrical heating. The desirable effect is obtained not by heating alone, but by the action of the magnetic field of the 95 alternating current on the molecular structure of the metal being treated.

The advantages of my invention result from the action of the magnetic field of an alternating current upon the metal. This 100 action is found to change the grain or molecular structure of the metal in different ways depending upon how the current is applied. That is, by varying the amount of current, the number of alternations per second, etc., the structure of the metal may be changed as desired. Other important advantages result from the uniform and regular heating of all parts of the metal, the accurate regulation of the temperature by 105 110

means of the current, the ease of reproducing the determining temperatures and the complete control of either rise or fall in temperature. The metal may be easily protected 5 from oxygen or other injurious gases during treatment. The increased fining effect on the metal over that of ordinary heat treatment or mechanical work can be easily determined by tests.

10 I attribute the benefits obtained by my process to the effect of the vibrations produced by the magnetic field of the alternating current, and the alterations in dimensions of the piece caused by it, but it is, of 15 course understood that, having determined by experiment that it gives improved results, I do not wish to limit myself to any theory as to the rationale of the process.

Another advantage of my process is that it 20 may be easily arranged to give automatic treatment without the necessity of personal supervision. Thus, in some of my experiments, I have placed a circuit breaker in the feed wire. In this case as the permeability 25 of the metal being treated to the magnetic flux decreases, the amount of the current increases up to a predetermined point and the circuit breaker thereupon automatically cuts it off. The current may be reestablished 30 and gradually lowered if desired, or the metal may cool slowly in the original envelop. If this is not desired, the article may be immediately withdrawn and 35 quenched. In this case, cutting off the current shows that the magnetic field has produced the proper effect and that the temperature has reached the desired point, thus giving a temperature regulation as well as 40 automatic completion of the process, where it is not desired to cool under the influence of the magnetic field.

It will be noted that my process is entirely 45 different from that of heating metals either by an induction furnace or by a heating coil. In the induction furnace, the metal under treatment is not subjected to the action of the magnetic field of an alternating current and the induced currents circulate in a special coil to the secondary of the furnace; 50 whereas in my process the induced currents circulate in the solid metal under treatment, which metal carries the magnetic field.

In the ordinary resistance heater, heat is 55 radiated from the resistance material to the metal being treated. In the use of my process, on the contrary, heat is generated in the metal which is being treated and inci-

dently radiates from it to the conductor carrying the currents.

My method not only produces a superior 60 product, but is capable of competing with present commercial methods of treating metals even at the present price of electric current, because the current is efficiently applied. Even as a method of heating it is 65 efficient because of the heat being generated throughout the material being treated instead of being conducted and radiated to it. This method also aids in giving a superior 70 character of product on account of uniform heating throughout the metal being treated.

Many changes may be made in the form 75 of apparatus employed as well as in the metal or alloy being treated, so long as the latter is in solid form, without departing from my invention. By solid metal I mean metal which is not in a molten condition.

I claim:

1. The method of treating solid metal to 80 alter its molecular structure, consisting in temporarily subjecting it to the action of the magnetic field of an alternating electric current, and protecting the metal against oxidation during such treatment.

2. The method of treating solid metal to 85 alter its molecular structure, consisting in heating it and at the same time subjecting it to the action of the magnetic field of an alternating current.

3. The method of treating solid metal to 90 alter its molecular structure, consisting in heating it by means of induced electric currents set up therein and simultaneously subjecting it to the action of the magnetic field of an alternating current.

4. The method of treating solid metal to 95 alter its molecular structure, consisting in temporarily subjecting it to the action of the magnetic field of an alternating current, and protecting the metal from the action of injurious gases during such treatment.

5. The method of treating solid metal to 100 alter its molecular structure, consisting in temporarily subjecting it to the action of the magnetic field of an alternating electric current, and protecting the metal against heat losses during such treatment.

In testimony whereof I have hereunto signed my name in the presence of the two 110 subscribed witnesses.

FREDERIC L. BISHOP.

Witnesses:

F. W. H. CLAY,  
FRED'K STAUB.